

# UNITED STATES PATENT OFFICE.

WILLIAM A. SALTER, OF KANSAS CITY, MISSOURI.

## PROCESS OF MANUFACTURE OF STEEL GUN AND ORDNANCE BARRELS.

1,199,430.

Specification of Letters Patent. Patented Sept. 26, 1916.

No Drawing.

Application filed December 10, 1915. Serial No. 66,096.

*To all whom it may concern:*

Be it known that I, WILLIAM A. SALTER, a citizen of the United States, residing at Kansas City, in the county of Jackson and 5 State of Missouri, have invented new and useful Improvements in the Process of Manufacture of Steel Gun and Ordnance Barrels.

This invention relates to the manufacture 10 of breech loading gun and ordnance barrels of steel composition, and has for its object, to render the process of turning out the completed barrel more expeditiously; to make a barrel in which the bursting or tensile 15 strength is greatly increased, and cheapen the cost of manufacture.

In the working of the steel, I take advantage of the fact that when it is heated to a red or a white heat, it expands considerably 20 over what it was in a cold state, and shrinks in cooling, and also while it is in a white or red heat stage, steel adapts itself to forging operations, by blows from hammers, rollers under pressure, or heavy pressure. 25 Also when a piece of steel is heated to a white or red heat to where it is in a semi ductile state and a strong cooling element is brought in contact with one side of it, that side of it will rapidly chill and the cooled 30 portion travel across the steel slowly until the entire piece is cooled. I employ these characteristics, and after turning the outside of my steel barrel to approximately its right size, and boring the hole throughout its

length, the barrel is brought to a heat where 35 it is adapted for working, and a strong cooling element such as water, or oil, or air under compression, is then forced through the bore, and as the bore starts to cool, the external part of the barrel is then subjected to 40 a compressing and reducing process, so that the hot exterior of the barrel is kept constantly compressed and reduced against the slowly cooling core around the bore, with the result that the completed barrel when, 45 cooled, is in a state of uniform compression around the bore, to resist the forces of explosion when in use.

I claim:

The process of manufacturing breech loading gun and ordnance steel barrels, consisting in preparing the barrel to approximately its right size having a bore throughout its length, heating the barrel to a working temperature, forcing a strong cooling medium through the bore, and as the walls of the bore start to cool, applying a prolonged compressing and reducing force to the external part of the barrel so that the hot exterior is kept compressed against the slowly 50 cooling walls of the bore, thus causing a uniform compression around the bore of the barrel, to resist the strain of expansion when 55 in use.

WILLIAM A. SALTER.

Witnesses:

GERHARD B. SCHROER,  
OLIVE A. SHORE.

Copies of this patent may be obtained for five cents each, by addressing the "Commissioner of Patents,  
Washington, D. C."